



US005962207A

# United States Patent [19]

Anderson et al.

[11] Patent Number: **5,962,207**[45] Date of Patent: **Oct. 5, 1999**[54] **MOTION PICTURE FILM**

[75] Inventors: **Charles C. Anderson**, Penfield; **Brian A. Schell**, Honeoye Falls; **Debasis Majumdar**, Rochester; **Mario D. DeLaura**, Hamlin, all of N.Y.

[73] Assignee: **Eastman Kodak Company**, Rochester, N.Y.

[21] Appl. No.: **09/018,867**

[22] Filed: **Feb. 5, 1998**

[51] Int. Cl.<sup>6</sup> ..... **G03C 1/85**; G03C 1/825; G03C 1/76

[52] U.S. Cl. ..... **430/517**; 430/510; 430/522; 430/527; 430/531; 430/536; 430/934; 430/961

[58] Field of Search ..... 430/527, 531, 430/536, 510, 517, 522, 934, 961

[56] **References Cited**

## U.S. PATENT DOCUMENTS

5,679,505 10/1997 Tingler et al. ..... 430/531

5,786,134 7/1998 Nalt et al. ..... 430/536

*Primary Examiner*—Richard L. Schilling*Attorney, Agent, or Firm*—Carl F. Ruoff[57] **ABSTRACT**

The present invention is a motion picture film including a support having on one side thereof an antihalation undercoat and at least one silver halide emulsion layer. The motion picture film has on the opposite side thereof an antistatic layer and a protective overcoat. The protective overcoat includes a layer of a polyurethane binder having a tensile elongation to break of at least 50% and a Young's modulus measured at a 2% elongation of at least 50000 lb/in<sup>2</sup>, and a topcoat farthest from said support. The topcoat is an interpolymer having repeating units of A and B wherein A is a fluorine containing acrylate or methacrylate monomer and B is an ethylenically unsaturated monomer containing hydratable groups.

**16 Claims, No Drawings**

## MOTION PICTURE FILM

CROSS REFERENCE TO RELATED  
APPLICATIONS

This application relates to commonly assigned copending application Ser. No. 09/019092, filed simultaneously herewith and hereby incorporated by reference for all that it discloses. This application relates to commonly assigned copending application Ser. No. 09/019093, filed simultaneously herewith and hereby incorporated by reference for all that it discloses.

## FIELD OF THE INVENTION

The present invention relates to an improved motion picture film, and more particularly to a motion picture film that resists tar adsorption and stain absorption.

## BACKGROUND OF THE INVENTION

Motion picture photographic films have long used a carbon black-containing layer on the backside of the film. This backside layer provides both antihalation protection and antistatic properties. The carbon black is applied in an alkali-soluble binder that allows the layer to be removed by a process that involves soaking the film in alkali solution, scrubbing the backside layer, and rinsing with water. This carbon black removal process, which takes place prior to image development, is both tedious and environmentally undesirable since large quantities of water are utilized in this film processing step. In addition, in order to facilitate removal during film processing, the carbon black-containing layer is not highly adherent to the photographic film support and may dislodge during various film manufacturing operations such as film slitting and film perforating. Carbon black debris generated during these operations may become lodged on the photographic emulsion and cause image defects during subsequent exposure and film processing.

After removal of the carbon black-containing layer the film's antistatic properties are lost. Undesired static charge build-up can then occur on processed motion picture film when transported through printers, projectors or on rewind equipment. Although these high static charges can discharge they cannot cause static marks on the processed photographic film. However, the high static charges can attract dirt particles to the film surface. Once on the film surface, these dirt particles can create abrasion or scratches or, if sufficiently large, the dirt particles may be seen on the projected film image.

In U.S. Pat. No. 5,679,505, incorporated herein by reference, a motion picture print film is described which contains on the backside of the support, an antistatic layer and a protective overcoat. The protective overcoat is comprised of a polyurethane binder and a lubricant. The polyurethane binder has a tensile elongation to break of at least 50% and a Young's modulus measured at 2% elongation of at least 50000 lb/in<sup>2</sup>. The tough, flexible overcoat has excellent resistance to abrasion and scratching during manufacture, printing, and projection, while acting as an effective processing barrier for the underlying antistatic layer.

However, post-processing tar deposits and stain have been a problem with protective overcoats in motion picture film. This tar is derived mostly from polymeric oxidized developer. The present invention relates to eliminating tar pickup during processing by providing a very thin topcoat over the polyurethane layer. The topcoat is obtained by the coating

and drying of a coating composition comprising an interpolymer containing at least two different segments; one of which is fluorinated and therefore oleophobic, the other of which is hydratable. The topcoat is effective at coverages so low that the excellent physical properties conferred upon the support by the polyurethane are retained.

## SUMMARY OF THE INVENTION

The present invention is a motion picture film including a support having on one side thereof an antihalation undercoat and at least one silver halide emulsion layer. The motion picture film has on the opposite side thereof an antistatic layer and a protective overcoat. The protective overcoat includes a layer of a polyurethane binder having a tensile elongation to break of at least 50% and a Young's modulus measured at a 2% elongation of at least 50000 lb/in<sup>2</sup>, and a topcoat farthest from said support. The topcoat is an interpolymer having repeating units of A and B wherein A is a fluorine containing acrylate or methacrylate monomer and B is an ethylenically unsaturated monomer containing hydratable groups.

DETAILED DESCRIPTION OF THE  
INVENTION

The photographic film support materials used in the practice of this invention are synthetic high molecular weight polymeric materials. These support materials may be comprised of various polymeric films, but polyester and cellulose triacetate film supports, which are well known in the art, are preferred. The thickness of the support is not critical. Support thickness of 2 to 10 mils (0.002–0.010 inches) can be employed, for example, with very satisfactory results. The polyester support typically employs an undercoat or primer layer between the antistatic layer and the polyester support. Such undercoat layers are well known in the art and comprise, for example, a vinylidene chloride/methyl acrylate/itaconic acid terpolymer or vinylidene chloride/acrylonitrile/acrylic acid terpolymer as described in U.S. Pat. Nos. 2,627,088, 2,698,235, 2,698,240, 2,943,937, 3,143,421, 3,201,249, 3,271,178 and 3,501,301.

The antihalation undercoat used in this invention functions to prevent light from being reflected into the silver halide emulsion layer(s) and thereby causing an undesired spreading of the image which is known as halation. Any of the filter dyes known to the photographic art can be used in the present invention as a means of reducing halation. Thus, for example, water-soluble dyes can be used for this purpose. Such dyes should be incorporated in the antihalation undercoat with a mordant to prevent dye diffusion.

Alternatively, and preferably, a solid particle filter dye is incorporated in the antihalation undercoat.

Useful water-soluble filter dyes for the purpose of this invention include the pyrazolone oxonol dyes of U.S. Pat. No. 2,274,782, the solubilized diaryl azo dyes of U.S. Pat. No. 2,956,879, the solubilized styryl and butadienyl dyes of U.S. Pat. Nos. 3,423,207 and 3,384,487, the merocyanine dyes of U.S. Pat. No. 2,527,583, the merocyanine and oxonol dyes of U.S. Pat. Nos. 3,486,897, 3,652,284 and 3,718,472, the enamino hemioxonol dyes of U.S. Pat. No. 3,976,661, the cyanomethyl sulfone-derived merocyanines of U.S. Pat. No. 3,723,154, the thiazolidones, benzotriazoles, and thiazolothiazoles of U.S. Pat. Nos. 2,739,888, 3,253,921, 3,250,617, and 2,739,971, the triazoles of U.S. Pat. No. 3,004,896, and the hemioxonols of U.S. Pat. Nos. 34,215,597 and 4,045, 229. Useful mordants are described, for example, in U.S. Pat. Nos. 3,282,699, 3,455, 693, 3,438,779, and 3,795,519.

Preferred examples of solid particle filter dyes for use in the antihalation underlayer of this invention are those described in U.S. Pat. No. 4,940,654. These solid particle filter dyes are compounds represented by the following formula(I):



where

D is a chromophoric light-absorbing moiety, which, when y is 0, comprises an aromatic ring free of carboxy substituents,

5

A is an aromatic ring, free of carboxy substituents, bonded directly or indirectly to D,  
X is a substituent, other than carboxy, having an ionizable proton, either on A or on an aromatic ring portion of D, having a pKa of about 4 to 11 in a 50/50 mixture (volume basis) of ethanol and water,

y is 0 to 4,

n is 1 to 7, and

the compound has a log partition coefficient of from about 0 to 6 when it is in unionized form.

Examples of filter dyes according to formula (1) include the following:



To promote adhesion of the antihalation underlayer to the support, primer layers as hereinabove described are advantageously employed, especially when the support is a polyester support.

The use of film-forming hydrophilic colloids as binders in photographic elements, including photographic films and photographic papers, is very well known. The most commonly used of these is gelatin and gelatin is a particularly preferred material for use in this invention it can be used as the binder in the antihalation underlayer and in the silver halide emulsion layer(s). Useful gelatins include alkali-treated gelatin (cattle bone or hide gelatin), acid-treated gelatin (pigskin gelatin) and gelatin derivatives such as acetylated gelatin, phthalated gelatin and the like. Other hydrophilic colloids that can be utilized alone or in combination with gelatin include dextran, gum arabic, zein, casein, pectin, collagen derivatives, collodion, agar-agar, arrowroot, albumin, and the like. Still other useful hydrophilic colloids are water-soluble polyvinyl compounds such as polyvinyl alcohol, polyacrylamide, poly(vinylpyrrolidone), and the like.

The photographic elements of the present invention can be simple black-and-white or monochrome elements or they can be multilayer and/or multicolor elements.

Color photographic elements of this invention typically contain dye image-forming units sensitive to each of the three primary regions of the spectrum. Each unit can be comprised of a single silver halide emulsion layer or of multiple emulsion layers sensitive to a given region of the spectrum. The layers of the element, including the layers of the image-forming units, can be arranged in various orders as is well known in the art.

A preferred photographic element according to this invention comprises at least one blue-sensitive silver halide emulsion layer having associated therewith a yellow image dye-providing material, at least one green-sensitive silver halide emulsion layer having associated therewith a magenta image dye-providing material and at least one red-sensitive silver halide emulsion layer having associated therewith a cyan image dye-providing material.

In addition to an antihalation underlayer and one or more emulsion layers, the elements of the present invention can contain auxiliary layers conventional in photographic elements, such as overcoat layers, spacer layers, filter layers, interlayers, pH lowering layers (sometimes referred to as acid layers and neutralizing layers), timing layers, opaque reflecting layers, opaque light-absorbing layers and the like.

The light-sensitive silver halide emulsions employed in the photographic elements of this invention can include coarse, regular or fine grain silver halide crystals or mixtures thereof and can be comprised of such silver halides as silver chloride, silver bromide, silver bromoiodide, silver chlorobromide, silver chloroiodide, silver chorobromoiodide, and mixtures thereof. The emulsions can be, for example, tabular grain light-sensitive silver halide emulsions. The emulsions can be negative-working or direct positive emulsions. They can form latent images predominantly on the surface of the silver halide grains or in the interior of the silver halide grains. They can be chemically and spectrally sensitized in accordance with usual practices. The emulsions typically will be gelatin emulsions although other hydrophilic colloids can be used in accordance with usual practice. Details regarding the silver halide emulsions are contained in *Research Disclosure*, Item 36544, September, 1994, and the references listed therein.

The photographic silver halide emulsions utilized in this invention can contain other addenda conventional in the

photographic art. Useful addenda are described, for example, in *Research Disclosure*, Item 36544, September, 1994. Useful addenda include spectral sensitizing dyes, desensitizers, antifoggants, masking couplers, DIR couplers, DIR compounds, antistain agents, image dye stabilizers, absorbing materials such as filter dyes and UV absorbers, light-scattering materials, coating aids, plasticizers and lubricants, and the like.

Depending upon the dye-image-providing material employed in the photographic element, it can be incorporated in the silver halide emulsion layer or in a separate layer associated with the emulsion layer. The dye-image-providing material can be any of a number known in the art, such as dye-forming couplers, bleachable dyes, dye developers and redox dye-releasers, and the particular one employed will depend on the nature of the element, and the type of image desired.

Dye-image-providing materials employed with conventional color materials designed for processing with separate solutions are preferably dye-forming couplers; i.e., compounds which couple with oxidized developing agent to form a dye. Preferred couplers which form cyan dye images are phenols and naphthols. Preferred couplers which form magenta dye images are pyrazolones and pyrazolotriazoles. Preferred couplers which form yellow dye images are benzoylacetanilides and pivaloylacetanilides.

Protective overcoats of the present invention may be successfully employed with a variety of antistatic layers well known in the art. The antistatic layer of this invention may include a variety of electrically conductive metal-containing particles, such as metal oxides, dispersed in a binder material. Many of these metal oxide particles do not require chemical barriers to protect them against harsh environments, such as photographic processing solutions. However, since many of these metal oxides require high particle loading in a binder to obtain good conductivity, i.e. antistatic properties, the physical properties are degraded and an abrasion resistant topcoat is required for good physical durability of the layers. Examples of useful electrically conductive metal-containing particles include donor-doped metal oxides, metal oxides containing oxygen deficiencies, and conductive nitrides, carbides, and borides. Specific examples of particularly useful particles include conductive  $TiO_2$ ,  $SnO_2$ ,  $V_2O_5$ ,  $Al_2O_3$ ,  $ZrO_2$ ,  $In_2O_3$ ,  $ZnO$ ,  $ZnSb_2O_6$ ,  $InSbO_4$ ,  $TiB_2$ ,  $ZrB_2$ ,  $NbB_2$ ,  $TaB_2$ ,  $CrB$ ,  $MoB$ ,  $WB$ ,  $LaB_6$ ,  $ZrN$ ,  $TiN$ ,  $WC$ ,  $HfC$ ,  $HfN$ , and  $ZrC$ . Examples of the patents describing these electrically conductive particles include; U.S. Pat. Nos. 4,275,103, 4,394,441, 4,416,963, 4,418,141, 4,431,764, 4,495,276, 4,571,361, 4,999,276, 5,122,445 and 5,368,995. Also included are:

Semiconductive metal salts such as cuprous iodide as described in U.S. Pat. Nos. 3,245,833, 3,428,451, and 5,075,171.

Fibrous conductive powders comprising, for example, antimony-doped tin oxide coated onto non-conductive potassium titanate whiskers as described in U.S. Pat. Nos. 4,845,369 and 5,116,666.

Conductive polymers, such as, the cross-linked vinylbenzyl quaternary ammonium polymers of U.S. Pat. No. 4,070,189 or the conductive polyanilines of U.S. Pat. No. 4,237,194.

A colloidal gel of vanadium pentoxide or silver-doped vanadium pentoxide as described in U.S. Pat. Nos. 4,203,769, 5,006,451, 5,221,598 and 5,284,714.

However, the preferred antistatic layer contains vanadium pentoxide as described in one of the aforementioned patents. The antistatic layer described in U.S. Pat. No. 4,203,769 is

prepared by coating an aqueous colloidal solution of vanadium pentoxide. Preferably, the vanadium pentoxide is doped with silver. A polymer binder, such as a cationic vinylidene-chloride-containing terpolymer latex or a polyesterionomer dispersion, is preferably employed in the antistatic layer to improve the integrity of the layer and to improve adhesion to the undercoat layer. Typically the dried coating weight of the vanadium pentoxide antistatic material is about 0.5 to 30 mg/m<sup>2</sup>. The weight ratio of polymer binder to vanadium pentoxide can range from about 1:5 to 500:1, but, preferably 1:1 to 10:1. Typically, the antistatic layer is coated at a dry coverage of from 1 to 400 mg/m<sup>2</sup> based on total dry weight. The electrical resistivity of the antistatic layer is preferably from about 7 to about 11 log Ω/sq, and most preferably less than 9 log Ω/sq.

The antistatic coating formulation may also contain a coating aid to improve coatability. The common level of coating aid in the antistatic coating formula is 0.01 to 0.30 weight percent active coating aid based on the total solution weight. However, the preferred level of coating aid is 0.02 to 0.20 weight percent active coating aid based on total solution weight. These coating aids can be either anionic or nonionic coating aids such as paraisononyloxy-glycidol ethers, octylphenoxy polyethoxy ethanol, sodium salt of alkylaryl polyether sulfonate, and dioctyl esters of sodium sulfosuccinic acid, which are commonly used in aqueous coatings. The coating may be applied onto the film support using coating methods well known in the art such as hopper coating, skim pan/air knife, gravure coating, and the like.

The antistatic layer of this invention is overcoated with a polyurethane. Preferably, the polyurethane is an aliphatic polyurethane. Aliphatic polyurethanes are preferred due to their excellent thermal and UV stability and freedom from yellowing. The polyurethanes of the present invention are characterized as those having a tensile elongation to break of at least 50% and a Young's modulus measured at an elongation of 2% of at least 50,000 lb/in<sup>2</sup>. These physical property requirements insure that the overcoat layer is hard yet tough to simultaneously provide excellent abrasion resistance and outstanding resiliency to allow the topcoat and antistat layer to survive hundreds of cycles through a motion picture projector. The polyurethane overcoat is preferably coated from a coating formula containing from about 0.5 to about 10.0 weight percent of polymer to give a dry coverage of from about 50 to about 3000 mg/m<sup>2</sup>. The dry coverage of the overcoat layer is preferably from about 300 to 2000 mg/m<sup>2</sup>.

The polyurethane may be either organic solvent soluble or aqueous dispersible. For environmental reasons, aqueous dispersible polyurethanes are preferred. Preparation of aqueous polyurethane dispersions is well-known in the art and involves chain extending an aqueous dispersion of a prepolymer containing terminal isocyanate groups by reaction with a diamine or diol. The prepolymer is prepared by reacting a polyester, polyether, polycarbonate, or polyacrylate having terminal hydroxyl groups with excess polyfunctional isocyanate. This product is then treated with a compound that has functional groups that are reactive with an isocyanate, for example, hydroxyl groups, and a group that is capable of forming an anion, typically this is a carboxylic acid group. The anionic groups are then neutralized with a tertiary amine to form the aqueous prepolymer dispersion. The chemical resistance of the polyurethane overcoat can be improved by adding a crosslinking agent that reacts with functional groups present in the polyurethane, for example, carboxyl groups. Crosslinking agents such as aziridines, carbodiimides, epoxies, and the like are suitable for this

purpose. The crosslinking agent can be used at about 0.5 to about 30 weight percent based on the polyurethane. However, a crosslinking agent concentration of about 2 to 12 weight percent based on the polyurethane is preferred.

The present invention includes a topcoat over the polyurethane overcoat to reduce or eliminate tar pickup. The topcoat contains a vinylic interpolymers having repeat units of A and B where A is derived from fluorine-containing acrylate or methacrylate monomers and B is derived from ethylenically unsaturated monomers containing hydratable groups.

More specifically, the unit A is derived from a fluoro(meth)-acrylate or mixture of fluoro(meth)acrylates represented by the following formula:



where the R<sub>f</sub> substituent is a monovalent, fluorinated, aliphatic organic radical having at least one carbon atom and as many as 20 carbon atoms, preferably, 2 to 10 carbon atoms. The skeletal chain of R<sub>f</sub> can be straight, branched, or cyclic, and can include catenary divalent oxygen atoms or trivalent nitrogen atoms bonded only to carbon atoms. Preferably, R<sub>f</sub> is fully fluorinated, but carbon-bonded hydrogen or chlorine atoms can be present as substituents on the skeletal chain of R<sub>f</sub>. Preferably, R<sub>f</sub> contains at least a terminal perfluoromethyl group. Preferably, p is 1 or 2.

The linking group L is a bond or hydrocarbyl radical linkage group containing from 1 to 12 carbon atoms and optionally substituted with and/or interrupted with a substituted or unsubstituted heteroatom such as O, P, S, N. R is either H or methyl. Preferably, the fluoro(meth)acrylate monomer contains at least 30 weight percent fluorine.

Non-limiting examples of fluoro(meth)acrylates useful in the present invention include:



where x is 0 to 20, preferably 2 to 10, y is 1 to 10, and R is H or methyl



where x is 0 to 20, preferably 2 to 10, y is 1 to 10, and R is H or methyl



where x is 0 to 20, preferably 2 to 10, y is 1 to 10, z is 1 to 4, R' is alkyl or arylalkyl, and R'' is H or methyl



where x is 1 to 7, y is 1 to 10, and R is H or methyl



where x+y is at least 1 up to 20, z is 1 to 10, and R is H or methyl.

The B unit is derived from ethylenically unsaturated monomers containing hydratable, ionic groups or hydratable, nonionic groups or combinations thereof. Examples of monomers containing ionic groups include

mono- or multifunctional carboxylic acid-containing molecules represented by the following formula:



where R is H, methyl, ethyl, carboxy, carboxymethyl, or cyano, L is a bond or hydrocarbyl radical linkage group containing from 1 to 12 carbon atoms and optionally substituted with and/or interrupted with a substituted or unsubstituted heteroatom such as O, P, S, N. x is equal to 1 or 2. This acid may be present in its protonated form or as its salt after neutralization with an organic or inorganic base.

The B unit may also be derived from ethylenically unsaturated monomers containing sulfonic acid groups, such as vinyl sulfonic acid, styrene sulfonic acid, 2-acrylamido-2-methyl propane sulfonic acid, and the like. Alternatively, the B unit may be derived from ethylenically unsaturated monomers containing phosphorous acid or boron acid groups. These may be present in their protonated acid or salt form.

The B unit may be derived from substituted or unsubstituted ammonium monomers such as N,N,N-trialkylammonium methyl styrene, N,N,N-trialkylammonium alkyl(meth)acrylate, N,N,N-trialkylammonium (meth)acrylamide, etc., where the counterion may be fluoride, chloride, bromide, acetate, propionate, laurate, palmate, stearate, etc.

The B unit may further be derived from ethylenically unsaturated monomers containing nonionic, hydrophilic groups. Suitable monomers include: mono- or multifunctional hydroxyl containing monomers such as hydroxyalkyl (meth)acrylates and N-hydroxyalkyl(meth)acrylamides; poly (oxyalkylene)-containing (meth)acrylates and poly (oxyalkylene)-containing itaconates, (meth)acrylamide, and vinyl pyrrolidone.

Preferably, the monomer containing nonionic, hydrophilic groups is a (meth)acrylate containing a poly(oxyalkylene) group in which the oxyalkylene unit has 2 to 4 carbon atoms, such as  $-\text{OCH}_2\text{CH}_2-$ ,  $-\text{OCH}_2\text{CH}_2\text{CH}_2-$ ,  $-\text{OCH}(\text{CH}_3)\text{CH}_2-$ , or  $-\text{OCH}(\text{CH}_3)\text{CH}(\text{CH}_3)-$ . The oxyalkylene units in said poly(oxyalkylene) being the same, as in poly (oxypropylene), or present as a mixture, as in a heteric straight or branched chain of blocks of oxyethylene units and blocks of oxypropylene units. The poly(oxyalkylene) group contains 4 to about 200, preferably, 5 to about 150 oxyalkylene units. A representative example of a poly (oxyalkylene)-containing meth(acrylate) suitable for the purpose of the present invention is represented by the following formula:



where R' and R'' are independently H or methyl, and x is 4 to 200.

The fluoro(meth)acrylate interpolymers of the invention comprise 10 to 90 wt % of units A and 10 to 90 weight % of units B. Non-interfering amounts of monomers other than those described above can also be incorporated into the fluoro(meth)acrylate interpolymers of this invention. For example, the interpolymers of this invention can contain up to about 50 weight percent of polymer units derived from ethylene, vinyl acetate, vinyl halide, vinylidene halide, acrylonitrile, methacrylonitrile, alkyl acrylates and methacrylates, glycidyl acrylate, glycidyl methacrylate, styrene, alkyl styrenes, vinylpyridine, vinyl alkyl ethers, vinyl alkyl ketones, butadiene, vinyl silanes, and mixtures thereof.

The fluoro(meth)acrylate interpolymers of the invention may be random, graft, or block copolymers. The molecular

weight of the interpolymers may be from about 5000 to about 10,000,000.

The stain resistant overcoat layers of the present invention may comprise the fluoro(meth)acrylate interpolymer in combination with another polymer. In a preferred embodiment, the other polymer is a water soluble or water dispersible polymer. Water soluble polymers include, for example, gelatin, polyvinyl alcohol, polyvinyl pyrrolidone, cellulosics, polystyrene sulfonic acid and its alkali metal salts or ammonium salts, water soluble (meth)acrylic interpolymers, and the like. Water dispersible polymers that may be used in conjunction with the fluoro(meth)acrylate interpolymer include latex interpolymers containing ethylenically unsaturated monomers such as acrylic and methacrylic acid and their esters, styrene and its derivatives, vinyl chloride, vinylidene chloride, butadiene, acrylamides and methacrylamides, and the like. Other water dispersible polymers that may be used include polyurethane and polyester dispersions. Preferably, the stain resistant overcoat layer contains at least 70 weight % of the fluoro(meth)acrylate interpolymer.

The stain resistant overcoat layer compositions in accordance with the invention may also contain suitable crosslinking agents including aldehydes, epoxy compounds, polyfunctional aziridines, vinyl sulfones, methoxyalkyl melamines, triazines, polyisocyanates, dioxane derivatives such as dihydroxydioxane, carbodiimides, and the like. The crosslinking agents may react with the functional groups present on the fluoro(meth)acrylate interpolymer, and/or the other water soluble or water dispersible polymer present in the coating composition.

The topcoat may additionally contain fillers for improving the modulus of the layer, lubricants, and additives such as matte beads for controlling the ferotyping characteristics of the surface.

Examples of reinforcing filler particles include inorganic powders with a Mohs scale hardness of at least 6. Specific examples are metal oxides such as g-aluminum oxide, chromium oxide, (e.g.,  $\text{Cr}_2\text{O}_3$ ), iron oxide (e.g., alpha- $\text{Fe}_2\text{O}_3$ ), tin oxide, doped tin oxide, such as antimony or indium doped tin oxide, silicon dioxide, aluminosilicate and titanium dioxide; carbides such as silicon carbide and titanium carbide; and diamond in fine powder.

A suitable lubricating agent can be included to give the topcoat a coefficient of friction that ensures good transport characteristics during manufacturing and customer handling of the photographic film. Many lubricating agents can be used, including higher alcohol esters of fatty acids, higher fatty acid calcium salts, metal stearates, silicone compounds, paraffins and the like as described in U.S. Pat. Nos. 2,588,756, 3,121,060, 3,295,979, 3,042,522 and 3,489,567. For satisfactory transport characteristics, the lubricated surface should have a coefficient of friction of from 0.10 to 0.40. However, the most preferred range is 0.15 to 0.30. If the topcoat coefficient of friction is below 0.15, there is a significant danger that long, slit rolls of the photographic film will become unstable in storage or shipping and become telescoped or dished, a condition common to unstable film rolls. If the coefficient of friction is above 0.30 at manufacture or becomes greater than 0.30 after photographic film processing, a common condition of non-process surviving topcoat lubricants, the photographic film transport characteristics become poorer, particularly in some types of photographic film projectors.

Aqueous dispersed lubricants are strongly preferred since lubricants, in this form, can be incorporated directly into the aqueous protective topcoat formula, thus avoiding a sepa-

rately applied lubricant overcoat on the protective topcoat layer. The aqueous dispersed lubricants of carnauba wax, polyethylene oxide, microcrystalline wax, paraffin wax, silicones, stearates and amides work well as incorporated lubricants in the aqueous, protective topcoat. However, the aqueous dispersed lubricants of carnauba wax and stearates are preferred for their effectiveness in controlling friction at low lubricant levels and their excellent compatibility with aqueous binders.

In addition to lubricants, matting agents are important for improving the transport of the film on manufacturing, printing, processing, and projecting equipment. Also, these matting agents can reduce the potential for the protective overcoat to ferrotype when in contact with the emulsion side surface under the pressures that are typical of roll films. The term "ferrotyping" is used to describe the condition in which the backside protective topcoat, when in contact with the emulsion side under pressure, as in a tightly wound roll, adheres to the emulsion side sufficiently strongly that some sticking is noticed between the protective topcoat and the emulsion side surface layer when they are separated. In severe cases of ferrotyping, damage to the emulsion side surface may occur when the protective topcoat and emulsion side surface layer are separated. This severe damage may have an adverse sensitometric effect on the emulsion.

The topcoat of the present invention may contain matte particles. The matting agent may be silica, calcium carbonate, or other mineral oxides, glass spheres, ground polymers and high melting point waxes, and polymeric matte beads. Polymeric matte beads are preferred because of uniformity of shape and uniformity of size distribution. The matte particles should have a mean diameter size of about 0.5 to about 3 micrometers. However, preferably the matte particles have a mean diameter of from about 0.75 to about 2.5 micrometers. The matte particles can be employed at a dry coating weight of about 1 to about 100 mg/m<sup>2</sup>. The preferred coating weight of the matte particles is about 15 to about 65 mg/m<sup>2</sup>. The surface roughness (Ra, ANSI Standard B46.1, 1985) in microns should be in the range 0.010 to 0.060 to prevent ferrotyping of the emulsion surface. The preferred Ra value range is from 0.025 to 0.045 for best performance. If the Ra value is below 0.025, there is insufficient surface roughness to prevent slight emulsion surface marking from ferrotyping between the backing and emulsion. If the Ra value is above 0.045, there is sufficient surface roughness with these size matte particles to show some low level of emulsion granularity and loss of picture sharpness, especially under the very high magnifications typical of movie theater projection.

The above described additives, including lubricants, matte beads, and fillers can also be present in the underlying polyurethane overcoat.

The stain resistant overcoat layers of the present invention may be applied from coating formulations containing up to 20% total solids by coating methods well known in the art. For example, hopper coating, gravure coating, skim pan/air knife coating, spray coating, and other methods may be used with very satisfactory results. The coatings are applied as part of the motion picture film support manufacturing process and are dried at temperatures up to 150° C. to give a dry coating weight of about 1 mg/m<sup>2</sup> to about 5000 mg/m<sup>2</sup>, preferably, the dry coating weight is about 2 mg/m<sup>2</sup> to about 500 mg/m<sup>2</sup>. The interpolymers may be applied from solvent or water-based coating formulations. Preferably, the fluoro (meth)acrylate interpolymers of the invention are water soluble or water dispersible and are applied from a water-based formulation.

The present invention is illustrated by the following examples. However, it should be understood that the invention is not limited to these illustrative examples.

## EXAMPLES

The polyurethane overcoats used in the examples were composed of Sancure 898 (B. F. Goodrich Company) and contained 6 percent by weight (based on polymer) of an aziridine crosslinker.

### Preparation of support containing an antistatic formulation

A subbed polyester support was prepared by first applying a subbing terpolymer of acrylonitrile, vinylidene chloride and acrylic acid to both sides of the support before drafting and tentering so that the final coating weight was about 90 mg/m<sup>2</sup>.

An antistatic formulation consisting of the following components was prepared at 0.078% total solids:

|                                                                    |         |
|--------------------------------------------------------------------|---------|
| Terpolymer of acrylonitrile, vinylidene chloride and acrylic acid, | 0.094%  |
| Vanadium pentoxide colloidal dispersion, 0.57%                     | 4.972%  |
| Rohm & Haas surfactant,                                            | 0.212%  |
| Triton X-100, 10%                                                  |         |
| Demineralized water                                                | 94.722% |

The antistatic formulation was coated over the subbed polyester support on the side opposite to the antihalation layer to give a dry coating weight of about 12 mg/m<sup>2</sup>.

Comparative Sample A comprised the following: a protective overcoat formulation was applied over the antistat layer. The overcoat formulation consisted of the following components:

|                                                                  | Dry Coverage, mg/m <sup>2</sup> |
|------------------------------------------------------------------|---------------------------------|
| Polyurethane dispersion, 32%                                     | 972                             |
| Carnauba wax dispersion,                                         | 0.65                            |
| Michelmlube 160, 25% (Michelman Inc.)                            |                                 |
| Matte, polymethyl methacrylate beads, 1.47 $\mu$ m, 23.8%        | 26.9                            |
| Polyfunctional aziridine crosslinker CX-100, (Zeneca Resins) 50% | 60.8                            |
| Rohm & Haas surfactant,                                          |                                 |
| Triton X-100, 10%                                                | 10.8                            |

A urethane overcoat identical to Comparative Sample A—excepting the carnauba wax was omitted—was prepared and the topcoats described in Table 1 were applied. All coatings contained 0.06% active Triton X-100 as coating aid.

Comparative Sample B comprised the carboxylic acid-functional perfluoropolyether described in commonly assigned copending application Ser. Nos. 08/932,014 and 08/932,597. Comparative Sample C comprised a fluorosurfactant having the formula

CF<sub>3</sub>(CF<sub>2</sub>)<sub>7</sub>SO<sub>2</sub>N(CH<sub>2</sub>CH<sub>3</sub>)CH<sub>2</sub>COO(CH<sub>2</sub>CH<sub>2</sub>O)<sub>40</sub>H and a hexamethoxymethyl melamine crosslinking agent (Cymel 303 Resin, Cytec Industries Inc.) Examples 1 and 2 comprised copolymers of a polyoxyalkylene acrylate and a perfluoroalkyl(meth)acrylate available from the 3M Company under the tradenames Scotchban FC-808 and FC-829A, respectively. Examples 3–7 comprised a fluoro(meth)acrylate containing anionic groups, nonionic, hydrophilic groups, and silanol groups available under the tradename Fluorad FC-759 from 3M Company.

## Tar Test

During routine film development, by-products of oxidized color developer will form brown, oily residue that may be adsorbed by the film surface and may create permanent, brown stained spots, i.e. tar.

A simulated developer tar test was performed on the samples to determine their propensity for tar/stain build-up. The test was done at 42° C. and involved smearing tar harvested from a developer tank onto the coating immersed in a developer bath followed by removal of the tar using dilute sulfuric acid. The resultant stain or tar is indicative of the propensity of the coating for tar adsorption. The resistance to tar stain was visually rated on a scale of 1 to 5, with 1 being the best performance, (i.e., no tar stain) and 5 being the worst performance (i.e., severe tar stain). The results are tabulated in Table 1.

TABLE 1

| Coating                                                             | Composition | Dry Coverage mg/m <sup>2</sup> | Tar Stain Rating |
|---------------------------------------------------------------------|-------------|--------------------------------|------------------|
| Comparative Polyurethane Sample A                                   |             | 1076                           | 5                |
| Comparative Fomblin Fluorolink "C" Sample B (Ausimont USA, Inc.)    |             | 10                             | 4                |
| Comparative Fluorad FC-431 Sample C (3M Company)                    |             | 50                             | 5                |
| Example 1 Scotchban FC-808 (3M Company)                             |             | 150                            | 2                |
| Example 2 Scotchban FC-829A (3M Company)                            |             | 150                            | 1                |
| Example 3 Fluorad FC-759 (3M Company)                               |             | 100                            | 1                |
| Example 4 Fluorad FC-759                                            |             | 50                             | 1                |
| Example 5 Fluorad FC-759                                            |             | 20                             | 1                |
| Example 6 Fluorad FC-759                                            |             | 5                              | 1                |
| Example 7 Fluorad FC-759 w/10 wt % CX-100 aziridine (Zeneca Resins) |             | 5                              | 1                |

As shown in Comparative Sample A, the polyurethane coating has very poor resistance to picking up developer tar, as do the fluoropolymers of Comparative Samples B and C. In contrast, the coatings of the invention exhibit excellent resistance to tar stain, even when employed as extremely thin layers relative to the underlying polyurethane. In addition, the coatings of the invention were transparent and had excellent adhesion to the polyurethane.

Additional stain resistant copolymers were prepared and evaluated in the following examples.

## Preparation of stain resistant copolymers

2.8 g FLUORAD fluorochemical acrylate FX-13 (3M Company), 1.6 g acrylic acid, 2.4 g poly(ethylene glycol) methacrylate, molecular weight equal to 360 (Aldrich), 1.2 g isobutyl methacrylate, 0.05 g azobisisobutyronitrile, and 32 g tetrahydrofuran were weighed into a 50 ml one-necked round-bottom flask. The contents were sparged with nitrogen for 10 minutes, after which the flask was sealed with a rubber septum and placed in a constant temperature bath at 65° C. After 24 hours, the solution was cooled to room temperature, neutralized with triethylamine, then diluted with 100 g distilled water. Tetrahydrofuran was removed via rotary evaporator to yield an 8% solution containing a polymer comprising 35 weight % FX-13, 20 weight % acrylic acid, 30 weight % poly(ethylene glycol) methacrylate, and 15 weight % isobutyl methacrylate. Additional copolymer compositions were prepared in an analogous manner and these polymers were used in the following examples.

Stain resistant topcoats were applied over the polyurethane protective overcoat that had been previously applied

over the antistat layer as described earlier. The stain resistant topcoats were then evaluated for tar stain resistance. The description of the copolymer compositions, coating compositions, and results obtained are given in Table 2.

TABLE 2

| Coating    | FX-13 | Copolymer Composition, weight % |                                    |                       |      | Dry Coverage, mg/m <sup>2</sup> | Tar Stain Rating |
|------------|-------|---------------------------------|------------------------------------|-----------------------|------|---------------------------------|------------------|
|            |       | Acrylic acid                    | Poly(ethylene glycol) methacrylate | Isobutyl Methacrylate |      |                                 |                  |
| Example 8  | 35    | 20                              | 30                                 | 15                    | 500  | 1                               |                  |
| Example 9  | 60    | 10                              | 30                                 | 0                     | 500  | 1                               |                  |
| Example 10 | 15    | 10                              | 30                                 | 45                    | 1000 | 3                               |                  |
| Example 11 | 45    | 10                              | 30                                 | 15                    | 1000 | 1                               |                  |
| Example 12 | 35    | 20                              | 30                                 | 15                    | 170  | 1                               |                  |
| Example 13 | 60    | 10                              | 30                                 | 0                     | 100  | 1                               |                  |

\* - all coatings contain 10 weight % CX100 aziridine crosslinking agent

The invention has been described in detail with particular reference to certain preferred embodiments thereof, but it will be understood that variations and modifications can be effected within the spirit and scope of the invention.

## What is claimed is:

1. A motion picture film comprising a support having, in order, on one side thereof an antihalation undercoat and at least one silver halide emulsion layer and having, in order, on the opposite side thereof an antistatic layer, a protective overcoat; comprising a layer of a polyurethane binder having a tensile elongation to break of at least 50% and a Young's modulus measured at a 2% elongation of at least 50000 lb/in<sup>2</sup>, and a topcoat farthest from said support overlying said layer of a polyurethane binder comprising an interpolymer having repeating units of A and B wherein A comprises a fluorine containing acrylate or methacrylate monomer and B comprises an ethylenically unsaturated monomer containing hydratable groups.
2. The motion picture film of claim 1, wherein said antihalation undercoat comprises a solid particle filter dye.
3. The motion picture film of claim 1, wherein said antistatic layer comprises electrically-conductive metal-containing particles selected from the group consisting of donor-doped metal oxides, metal oxides containing oxygen deficiencies, conductive nitrides, conductive carbides and conductive borides.
4. The motion picture film of claim 1, wherein said antistatic layer comprises an electrically-conductive polymer.
5. The motion picture film of claim 1, wherein said antistatic layer comprises vanadium pentoxide.
6. The motion picture film of claim 1, wherein said antistatic layer has a dry coverage of from 1 to 400 mg/m<sup>2</sup>.
7. The motion picture print film of claim 1, wherein said polyurethane binder is an aliphatic polyurethane.
8. The motion picture print film of claim 1, wherein said polyurethane binder is an aqueous-dispersible polyurethane.
9. The motion picture print film of claim 1, wherein A is represented by the following formula:



wherein R<sub>f</sub> is a monovalent, fluorinated, aliphatic organic radical having from one to 20 carbon atoms, p is 1 or 2, L is a bond or hydrocarbyl radical linkage group containing from 1 to 12 carbon atoms and R is either H or methyl.

**15**

**10.** The motion picture print film of claim 1, wherein B is represented by the following formula:



wherein R is hydrogen, methyl, ethyl, carboxy, carboxymethyl, or cyano, L is a bond or hydrocarbyl radical linkage group containing from 1 to 12 carbon atoms where x is 1 or 2.

**11.** The motion picture print film of claim 1, wherein B is an ethylenically unsaturated monomer containing sulfonic acid groups, phosphorous acid groups, boron acid groups, nonionic hydrophilic groups.

**12.** The motion picture print film of claim 1, wherein said interpolymer comprises from 10 to 90 wt % of units A and from 10 to 90 weight % of units B.

<sup>10</sup> **5.** **13.** The motion picture print film of claim 1, wherein said interpolymer further comprises ethylene, vinyl acetate, vinyl halide, vinylidene halide, acrylonitrile, methacrylonitrile, glycidyl acrylate, alkyl acrylate, alkyl methacrylate, glycidyl

methacrylate, styrene, alkyl styrene, vinylpyridine, vinyl alkyl ether, vinyl alkyl ketone, butadiene and vinyl silane.

**14.** The motion picture print film of claim 1, wherein said interpolymers have a molecular weight of from about 5000 to about 10,000,000.

**15.** The motion picture print film of claim 1, wherein said topcoat further comprises crosslinking agents.

**16.** The motion picture print film of claim 1, wherein said topcoat further comprises fillers, lubricants, or matte beads.

\* \* \* \* \*

**16**